

Aug. 1, 1939.

P. GÖRLICH

2,168,259

PHOTOELECTRICALLY RESPONSIVE LAYER

Original Filed May 3, 1937

Fig. 1



Fig. 3



Fig. 2



Fig. 4



Fig. 5



Inventor  
Paul Görlich  
By:  
B. Singer & F. Stern  
his Atty's.

## UNITED STATES PATENT OFFICE

2,168,259

PHOTOELECTRICALLY RESPONSIVE  
LAYER

Paul Görlich, Dresden, Germany, assignor to  
Zeiss Ikon Aktiengesellschaft, Dresden, Germany

Original application May 3, 1937, Serial No.  
140,449. Divided and this application August  
29, 1938, Serial No. 227,292. In Germany Feb-  
ruary 22, 1936

3 Claims. (Cl. 250—27.5)

The present invention is a division of my application for Letters Patent filed in the United States Patent Office on the 3rd day of May 1937, Serial No. 140,449, now patent numbered 2,140,994, relating to improvements in photoelectrically responsive layers and in particular to a method of producing minutely subdivided photoelectrically responsive layers upon carriers of any desired kind. Photoelectrically responsive layers of this type are employed particularly in television transmitting (dissectors) tubes.

Owing to the resemblance which this minute subdivision has with the surface of screen as used in printing processes they are referred to as "screen" areas in the following specification.

Television tubes frequently are provided with extensive photoelectrically responsive areas, and it has been found that the efficiency of these areas is enhanced if the same are minutely subdivided, to resemble in appearance that of an extremely fine mesh screen. Whenever a point of light strikes a "dot" of this photoelectrically responsive screen area electrical charges are instantly set up with the magnitude of the electric charge dependent upon the intensity of the light. These charges are utilized for modulating the television transmitter.

The production of screen layers of photoelectrically responsive material heretofore was very difficult, because it is necessary to make the individual layer sections extremely small. One method used heretofore consists in this, that an extremely thin silver coating is deposited by vaporization upon a carrier of insulating material in such manner, that the silver particles do not form a closely coherent area. Such incoherent layer, however, can be produced only under conditions that the silver coating is extremely thin so as to be almost transparent. Obviously, the photoelectric efficiency of such layers is very poor, because the greatest amount of light passes unrestricted through the layer.

It is now an object of the invention to eliminate the disadvantages of the known methods of this type.

Fig. 1 illustrates diagrammatically and highly magnified a plan view of a carrier base provided with finely distributed selenium dots in accordance with the first method step of the present invention.

Fig. 2 is a cross sectional view substantially along the line of 2—2 of Fig. 1, and the

Figs. 3, 4 and 5 are cross-sectional views similar to Fig. 2 and illustrate additional steps of the method of the invention.

The present invention makes use of the fact that selenium, particularly when in an extremely pure state, has a very high surface tension. It is possible to liquefy finely distributed selenium without the fine selenium droplets thus produced being of such low surface tension that they would immediately flow into each other.

This property of selenium is made use of by the present invention, for producing upon a carrier base innumerable point-like dots in extremely fine distribution. The base may be of conductive material, as for instance silver, or of non-conductive material. These dots are then rendered photoelectrically responsive by some subsequent treatment.

The selenium screens may be produced in various manners. It is for instance possible to mix the selenium with a floating agent, which may consist of any desired liquid, and to deposit the selenium from this mixture upon the carrier base. Another method, which may be used, consists in mixing finely divided selenium with a material which forms a paste with the selenium, and spreading this selenium containing paste upon the carrier base. The foreign material may then be removed from the selenium paste by steaming, dissolution, evaporation or the like.

A very practical method consists in depositing the selenium by condensation from vapor upon the carrier base. Contrary to expectation, it has been discovered that when employing the last named method, the selenium will not be deposited on the base in form of a coherent layer, but up to a substantial thickness of the layer it will be deposited in the form of small drops which are spaced from each other. Only when the selenium layer assumes a very great thickness the drops merge and form a coherent layer. In this respect selenium has similar properties as for instance mercury.

The Figs. 1 and 2 illustrate diagrammatically in a greatly magnified scale a carrier base consisting of a plate 1 of insulating material having a conductive surface coating 3, for instance silver, provided with finely distributed selenium dots 2 produced in any one of the just described manners.

In accordance with the present invention, the next step consists in the removal of the silver from those portions of the base which are not occupied by selenium droplets 2. This can be done, for instance, by etching. Fig. 3 illustrates a section of the carrier after the portions 3<sup>a</sup> (Fig. 2) of the silver layer 3 have been removed.

The agent for etching may be, e. g., sodium

thiosulphate, ammonia sulpho cyanide, nitric acid etc.

After the portion 3<sup>a</sup> of the metallic coating 3 between the selenium dots 2 have been removed the selenium is removed from the minute portions 3<sup>b</sup> of the metallic coating 3 which is covered. The removing of the selenium dots 2, which are used only temporarily as protection for the portions 3<sup>b</sup> of the metallic coating 3, is effected by 10 any suitable means of e. g. carbon-disulphide.

The metallic dots 3<sup>b</sup> are now exposed as shown in Fig. 4 and can now be made photoelectric sensitive by employing any known method. The minutely subdivided silver coating, for instance 15 may be oxidised and then be subjected to the action of light sensitive material, as caesium, whereby the dots of oxidised silver are covered with caesium. The resulting minutely subdivided 20 light sensitive layer composed of caesium dots 4 on oxidised silver dots 3<sup>b</sup> is illustrated in Figs. 5.

The oxidation is effected in known manner by a glow discharge in an atmosphere of oxygen, and the light sensitive metal, e. g., caesium is deposited by evaporation, thus forming the well known 25 bodies of Cs—O—Ag. The particles of caesium, deposited between the silver dots, are finally removed in known manner, e. g., by heating. This is possible owing to the fact that the adsorptive 30 forces of silver oxide against caesium is greater than the adsorptive forces of the layer itself.

The insulating carrier of the light sensitive layer may consist of glass, mica or other transparent material or if desired, of materials, which are not transparent.

35 What I claim as my invention is:

1. A method of producing a minutely subdivided photoelectrically responsive layer upon a carrier of insulating material provided with a metallic coating, including the steps of depositing on the 40 metallic coating of said carrier unfused selenium particles in sufficient quantity to produce from said selenium particles owing to their surface tension a screen-like layer composed of selenium

dots, removing those portions of the metallic coating from said carrier which are not covered by selenium dots, removing the selenium dots, thereby exposing those portions of the metallic coating formerly covered by selenium, and then 5 applying a photoelectrically responsive metal to the exposed dot-like portions of the screen-like metallic coating.

2. A method for producing a minutely subdivided photoelectrically responsive layer upon a carrier of insulating material provided with a metallic coating, including the steps of depositing on the metallic coating of said carrier by condensation from vapor unfused selenium particles in sufficient quantity to produce from said 15 selenium particles owing to their surface tension a screen-like layer composed of selenium dots, removing those portions of the metallic coating from said carrier which are not covered by selenium dots, removing the selenium dots, thereby exposing those portions of the metallic coating formerly covered by selenium, and then applying 20 a photoelectrically responsive metal to the exposed dot-like portions of the screen-like metallic coating.

25 3. A method of producing a minutely subdivided photoelectrically responsive layer upon a carrier of insulating material provided with a metallic coating, including the steps of depositing on the metallic coating of said carrier by condensation from vapor unfused selenium particles in sufficient quantity to produce from said selenium 30 particles owing to their surface tension a screen-like layer composed of selenium dots, removing those portions of the metallic coating from said carrier which are not covered by selenium dots, removing the selenium dots, thereby exposing those portions of the metallic coating formerly covered by selenium, oxidizing the screen-like 35 metallic coating, and then applying a photoelectrically responsive metal to the exposed dot-like portions of the screen-like metallic coating.

PAUL GÖRLICH.